

June 3, 1969

D. H. PREIST ET AL

3,448,413

R-F WINDOW FOR HIGH POWER ELECTRON TUBES

Original Filed April 16, 1962



Fig. 3



Fig. 4



Fig. 2

Fig. 1

INVENTORS  
DONALD H. PREIST  
RUTH CARLSON TALCOTT

BY

*Robert W. Dilts*

ATTORNEY

3,448,413

**R-F WINDOW FOR HIGH POWER  
ELECTRON TUBES**

Donald H. Preist, Mill Valley, and Ruth Carlson Talcott, Berkeley, Calif., assignors to Varian Associates, Palo Alto, Calif., a corporation of California  
Original application Apr. 16, 1962, Ser. No. 187,521, now Patent No. 3,252,034. Divided and this application Sept. 27, 1965, Ser. No. 490,204  
Int. Cl. H01p 1/00, 7/06

U.S. Cl. 333—98

4 Claims

**ABSTRACT OF THE DISCLOSURE**

Failure of windows transparent to radio-frequency electromagnetic energy due to single surface and two surface multipacting of electrons involving the window is described. Window structures including means for preventing such failure are disclosed and the manufacture of such structures and their incorporation into a radio frequency device, specifically a klystron, are described.

This application is a division of our co-pending application Ser. No. 187,521 filed Apr. 16, 1962, now Patent No. 3,252,034.

This invention relates to windows transparent to radio-frequency electromagnetic energy, and particularly to such windows fabricated in a manner to render them less susceptible to heating due to electron bombardment.

In the electron tube industry, one of the limiting factors determining the amount of power which can be extracted from an electron tube involves the output means for the tube. The output means is often in the form of dielectric material forming a "window" transparent to radio-frequency electromagnetic energy. The limiting factor is that the amount of power which a window is capable of passing has not kept pace with the amount of power which an electron tube is capable of generating. Thus, while it is possible with state-of-the-art electron tubes to generate very high powers, it is becoming increasingly difficult to extract such power from the electron tube because of the limitations imposed by the output means, especially where such output means is a dielectric window as used in micro-wave tubes such as klystrons, for instance.

Output windows transparent to electromagnetic energy are usually fabricated from dielectric materials having a coefficient of secondary electron emission greater than unity for values of an accelerating electric field greater than about 40-80 volts, and this characteristic renders them susceptible to destructive heating due to single surface multipacting by secondary electrons emitted from the window itself when the accelerating electric field exceeds a critical value. This phenomenon is explained at length in an article by the inventors herein, appearing in the IRE Transactions of the Professional Group on Electron Devices, vol. EE-8, No. 4, dated July 1961. It is therefore one of the objects of the invention to provide a composition of dielectric material which possesses a maximum coefficient of secondary emission of electrons of about unity or less for values of bombarding electron velocity at least several times higher than the usual range of 40-80 volts.

Another object of the invention is to provide an article of manufacture fabricated from a dielectric material having a maximum coefficient of secondary electron emission of not substantially more than unity under the conditions stated in the preceding paragraph.

Another of the important objects of the invention is to provide a radio-frequency output window fabricated from a material having a secondary electron emission coefficient of about or less than unity in the presence of free

electrons in vacuum and bombarding electron velocity substantially higher than 40-80 volts.

Still another object of the invention is the provision of an output window having a coefficient of secondary electron emission of about or less than unity and which also possesses thermal stress resistance sufficient to withstand temperature gradients caused by dielectric losses, for example, without failure due to fracture, softening, or chemical instability usually associated with such temperature gradients.

Still another important object of the invention is the provision of radio-frequency output window having a coefficient of secondary electron emission of about or less than unity, and which also possesses the requisite dielectric strength even at elevated temperatures to withstand very high voltage gradients.

A still further object of the invention is the provision of a high power radio-frequency output window for electron tubes which possesses chemical stability even when subjected to extremes in temperature such as during bake-out.

Still another object of the invention is the provision of a microwave structure incorporating such a window.

A still further object of the invention is the provision of a dielectric and metallic microwave structure incorporating a dielectric radio-frequency window fabricated from material treated to possess a secondary electron emission coefficient of about or less than unity in vacuum and in the presence of free electrons, and in which the metallic parts of the structure have also been treated so as to have a secondary electron emission coefficient of about or less than unity.

A still further object of the invention is to provide an electron tube having at least one resonant cavity portion equipped with at least one radio-frequency window which possesses a secondary electron emission coefficient of about or less than unity, and in which the conductive metallic walls of the resonant cavity also possess a secondary electron emission coefficient of about or less than unity.

The power-passing limitations which afflict radio-frequency windows are applicable alike to cylindrical and flat resonant cavity windows and also to flat and conical windows such as are used in waveguides. It is therefore another object of the invention to provide a microwave window assembly constructed in a manner to decrease electron bombardment of the window and thereby decrease the amount of heat generated in the window, and to dissipate by efficient conduction such heat as is generated in the window.

A still further object of the invention is the provision of a resonant cavity portion for a klystron tube in which the window is fabricated from a high thermal conductivity dielectric such as beryllia, and the associated metallic parts are fabricated from oxygen-free high-conductivity copper, with both the dielectric and metal portions of the cavity coated with a layer of metallic material which reduces to about or less than unity the coefficient of secondary electron emission from both the dielectric and metal parts.

The invention possesses other objects and features of value, some of which, with the foregoing, will be apparent from the following description and the drawings. It is to be understood, however, that the invention is not limited to the embodiments illustrated and described, but may be incorporated in varying forms within the scope of the appended claims.

Broadly considered, the invention in one of its aspects comprises the provision of a dielectric material having a coefficient of secondary electron emission of about or less than unity for values of bombarding electron velocity

at least several times higher than the usual range of 40-80 volts; and in another aspect the utilization of such material in combination with metallic bodies or surfaces which also have a secondary electron emission coefficient of about or less than unity to provide radio-frequency high-power output windows for microwave devices. It is well known in the art that dielectric materials suitable as high power output windows normally have, in the presence of charged particles, such as electrons, and high radio-frequency alternating electric fields, a coefficient of secondary electron emission substantially greater than unity. For alumina ceramics, for instance, the maximum secondary ratio is greater than 3. According to this invention the dielectric window material has been rendered less susceptible to secondary electron emission over a wider range of bombarding velocities by the application thereto of titanium by a method described and claimed in a copending application. The titanium is preferably incorporated in the dielectric material after the dielectric material has been fabricated into the desired configuration for use as an output window, but it is believed that such incorporation may also be effected during the manufacture of the dielectric material. In the former case, it has been found that titanium deposited on selected dielectric materials by vacuum deposition to a thickness of about 100 Angstrom units or less will result in a dielectric composition which retains the requisite dielectric strength to be used as a high-frequency, high-power output window, together with the other requisite characteristics pertaining to dielectric loss, thermal stress, and chemical stability, as discussed above. When incorporated in a metallic structure such as a resonant cavity or waveguide, the metallic structure is also provided with a layer of titanium, so that the secondary electron emission coefficient of the metallic surfaces will also be about or less than unity. Such a window construction has been found to be completely free from destructive heating due to secondary emission of electrons from the surface of the window itself, or from secondarily emitted electrons originating in the adjacent metallic structure.

Referring to the drawing:

FIGURE 1 is an elevation of a klystron tube incorporating a radio-frequency output window in accordance with the invention. The output window assembly is shown in vertical section.

FIGURE 2 is an enlarged vertical sectional view of that portion of FIGURE 1 indicated by the bracket 2. The titanium coatings on the interior surfaces are shown in exaggerated thickness for clarity.

FIGURE 3 is vertical sectional view through a waveguide portion equipped with a window according to this invention.

FIGURE 4 is a graph showing the secondary emission coefficient ( $\delta$ ) as a function of velocity (V) of bombarding electrons expressed in volts for coated and uncoated dielectric windows.

In the early days of UHF, when klystron tubes, for instance, were first coming into their own, radio-frequency transparent windows were almost exclusively made of glass, and were capable of handling only a few kilowatts of CW power. In such early klystron tubes, power output was limited by failure of the window in the output cavity, and such failure was ascribed to overheating of the glass window caused by dielectric losses in the window material. As the industry became more knowledgeable, ceramic materials having greater resistance to thermal stresses were substituted for glass materials. The geometries or configurations of associated metallic structures also changed in order to take advantage of ceramic materials. Ceramic windows enable reliable operation at the 10-kilowatt level at frequencies between 700 and 1,000 megacycles, and considerably higher power at lower frequencies. In the race to develop tubes of the klystron type having higher frequencies and higher output power, the assignee of the present invention pioneered

the utilization of external resonant cavities coupled to an electromagnetic field within the klystron envelope through a dielectric or ceramic window. A klystron tube of this type is illustrated, described and claimed in U.S. Patent No. 2,619,611, issued to the assignee of the present invention. As the power output increased from these new and better tubes, the limiting factor again became the tendency of the large output windows to rupture, thus destroying the envelope. Even integral cavity tubes, which utilized dielectric or ceramic windows interposed in a waveguide output, suffer from the inability of passing through the waveguide window the large power output from these tubes.

It was believed at the outset that the dielectric losses of the dielectric material itself, usually ceramic, caused heating of the ceramic material which resulted in rupture thereof. Such dielectric losses do of course cause heating, but usually not sufficient heating to rupture the window. Another theory that has been advanced to explain the rupturing of windows at high power outputs is that electrons from the electron beam or other source bombard the window and cause rupture. A still further theory is that secondary electrons, released from the metallic output gap drift tube assemblies by bombarding primaries of the beam, arrive at the window with high velocity, the kinetic energy of the electrons being transformed into heat on the window, and the window being caused to rupture as a result hereof. It has been found that under some special circumstances excessive multipacting at the output gap can cause such bombardment of the window, but in the usual case does not occur.

Through an extensive study program it has been determined that in the usual case heating and resultant rupture of dielectric output windows is caused by a phenomenon known as single surface multipacting on the surface of the dielectric material itself, triggered by an electron or electrons arriving at the window from within the envelope and impinging on the window with a force at least sufficient to liberate secondary electrons from the dielectric material. The phenomenon is called two-surface multipacting when the multipacting occurs between a waveguide surface and the adjacent surface of an inclined waveguide window, or between the diverging surfaces adjacent the apex end of a conical waveguide window. The triggering electrons do not usually come from the beam, but rather are emitted from adjacent metal parts as a result of the presence of high intensity electric fields. It has been found that the free secondary electrons liberated from the dielectric window material are accelerated to critical velocities by the alternating electric field adjacent the vacuum side of the window and are redirected toward the dielectric window such that additional free secondaries are liberated from the dielectric material when the accelerated and redirected free secondary electrons impinge on the dielectric window. As illustrated by the full line in the graph of FIGURE 4, for conventional uncoated or untreated radio-frequency windows, the critical field strength required to accelerate an electron sufficiently to commence single surface multipacting and heating as a result thereof corresponds to bombarding electron velocities ranging between 40 and 80 volts.

After considerable experimentation and analysis, it has been determined that by providing a coating or layer of some material on the inside surface of the dielectric material and adjacent metallic parts, composed of a material having a low secondary emission characteristic, beneficial results can be obtained in that the value of the critical field strength required to accelerate electrons to a bombarding velocity sufficient to commence single surface multipacting is greatly increased as shown by the dash line in the graph of FIGURE 4. At this higher critical field strength electrons starting from rest are accelerated  $(2n+1)$  half cycles to a bombarding velocity more than sufficient to release one secondary electron per bombard-

ing electron corresponding to a coefficient of secondary electron emission of unity on impact with a conventional window. As seen from the graph, the critical field strength has been increased so that it approaches the critical field strength at which maximum secondary emission occurs, with maximum secondary emission occurring at about or not substantially above unity, as shown. The realization of these beneficial results depended on the determination of a material to put on the dielectric and metal surfaces which would not have deleterious effects either on the electromagnetic transparency of the window or its dielectric loss, its chemical stability, its resistance to thermal stress, and which would not have the tendency of forming an oxide coating on interior metallic surfaces. Other important factors also had to be considered, such as the ability of the coating to withstand bakeout temperatures and to be uncontaminating to other associated parts.

In addition to the problem of determining what coating material to use, a secondary problem but of equal importance was the problem of determining the thickness of the coating or film and the method of its application. To be effective as an electromagnetic window, the dielectric material obviously must remain transparent to electromagnetic energy, and the interior surface of the window must therefore be nonconductive, or if conductive in some small degree, the dielectric loss of the material must remain within certain limits. Another problem was the method of controlling the thickness of the coating material so that the effects would be reproducible from one body to another, and from one electron tube to another. The method of application of such a coating, and the method of determining the thickness, has been described in a copending application.

It has been found that a body of dielectric material normally having in the presence of free electrons and a radio-frequency alternating electric field of sufficient intensity to accelerate the free electrons to a critical bombardment velocity where the coefficient of secondary emission of such electrons is greater than unity, may be transformed into a body of dielectric material having a coefficient of secondary emission of about or less than unit for a greatly expanded range of electric field intensities or bombarding velocities by application to one or all of its surfaces of an extremely thin coating or layer of titanium. This transformation is illustrated graphically in FIGURE 4 which at  $V_1$  indicates the usual critical field strength for conventional uncoated windows, and at  $V_2$  indicates the expanded range of field strength required before a critical value of bombardment velocity is reached. Titanium may be applied as a coating or layer on the window after its manufacture and formation into the requisite configuration, and it is believed the titanium may be incorporated in a surface zone of the dielectric material during the process of manufacture of specific window configurations from the dielectric material. In either case it is desirable that the coating or layer of titanium be of reproducible thickness, and that the electrical resistance of the dielectric material remain in the range between  $10^7$  to  $10^{11}$  ohms per square. It has been found that in order to maintain resistance of a dielectric body within the requisite range, a film is required which is so thin as to be invisible either on an opaque dielectric surface or on a transparent dielectric surface.

The secondary electron emission yield of an electrically conducting surface is determined by the composition of its surface to the depth of penetration of a bombarding primary electron. In a radio-frequency (R-F) device, the penetration depth is not very great since the velocity of electrons traveling in an R-F field is limited to that velocity which can be attained in one-half of one R-F cycle. In many practical devices, this does not exceed a few hundred volts at a dielectric surface and a few thousand volts in the higher voltage regions of a klystron or traveling wave tube, for instance. Accordingly, it has been found that films on the order of 1,000 Angstrom units of a dense

material such as titanium are sufficient to diminish to about or less than unity the secondary emission yield in the highest voltage regions of an electrically conducting surface, and that films 100 Angstrom units or less are adequate on dielectric surfaces to diminish the secondary emission yield to about or less than unity. In the case of the dielectric surface, however, the coating must be discontinuous in nature in order that the electrical resistance remain between  $10^7$  and  $10^{11}$  ohms per square. Such a discontinuous nature in the coating provides the high resistance while also providing the thickness required to control the secondary electron emitting characteristics of the surface.

In FIGURE 2 is illustrated the internal resonant cavity portion 2 from the external resonant cavity type klystron illustrated in FIGURE 1, which includes an electron gun section 4, a radio-frequency interaction section 6, and a collector section 7. As is well known in the art, the electron gun section, the radio-frequency section, and the collector section are hermetically united in axial alignment to enable the projection of an electron beam through a series of drift tube sections 8, each terminating within a cavity in a conically tapered end portion 9 spaced from the associated end of an adjacent drift tube section to provide an interaction gap 12 therebetween. Drift tube sections 8 are supported in axially spaced alignment by relatively heavy transversely extending annular metallic plates 13, preferably fabricated from oxygen-free high-conductivity copper. These plates, in turn, are held in axially spaced relationship by the cylindrical dielectric radio-frequency windows 14, one of which is designated as the output window. The opposite ends of the cylindrical dielectric windows are hermetically united to the associated drift tube supporting plates by sealing flange structures 16 described at greater length in United States Patent 2,903,614. Such a sealing structure introduces flexibility in the window design to accommodate differences in expansion and contraction of the dielectric window and the metallic drift tube and supporting plate assembly.

As illustrated in FIGURE 2, the inner surface 17 of the cylindrical dielectric window is provided with a thin coating or layer 18 of titanium, deposited thereon by the method described and claimed in a copending application. The coating is preferably deposited by vapor deposition of pure titanium metal in vacuum in a manner to provide a uniformly thick coating of titanium over the inner surface of the dielectric window. To complete the cavity, the adjacent metallic surfaces 19 of the drift tube supporting plates, the conical metallic surfaces 21 of the drift tube tips within the cavity, and a portion of the surface 22 forming the inner bore of each drift tube tip, are coated with a layer 23 of pure titanium metal to a thickness of about one-tenth of a mil. In FIGURE 2 the layer of titanium on these surfaces is exaggerated in thickness for clarity.

Experience has taught that a layer of titanium on these surfaces somewhat less than one-tenth of a mil thick is satisfactory and will reduce the secondary electron emission coefficient of these metal parts to a value of about or less than unity for values of electric fields at which other characteristics, such as external arc-over, become limiting factors. Because coatings of such scant thicknesses are difficult to measure, it has been found that when the characteristically copper-colored parts are completely opaque to visual inspection due to the deposition thereon of pure titanium, the coated metallic parts will appear grey and the thickness of the titanium will be adequate to provide the requisite low secondary electron emission characteristic. It will of course be understood that where desirable, any or all windows of the klystron, in addition to other dielectric bodies, such as the electron gun ceramics, may be coated with titanium with beneficial results. It should also be understood that the metallic surfaces within the evacuated envelope of an integral cavity klystron, including a waveguide output having a

flat output window, may be coated as described with beneficial results.

In FIGURE 3 is illustrated a flat circular dielectric waveguide window 26 having its periphery 27 hermetically united to the inner surface 28 of a metallic waveguide 29. One surface of the window is provided with a layer 31 of titanium about 100 Angstrom units thick, while the adjacent inner metallic surface of the waveguide is provided with a coating 32 of titanium at least 1,000 Angstrom units thick, or in the alternative, about one-tenth of a mil.

Regarding choice of materials, it is preferred that the metallic elements of the combination be fabricated from oxygen-free high-conductivity copper, and that the dielectric materials be selected from the group including fused silica, alumina-silicate glass, steatite, forsterite, alumina, beryllia or pyroceram. Materials selected from this group will be found to have a dielectric constant ranging from about 3.8 for fused silica to about 8 or 9 for alumina. In terms of the power factor or loss tangent, it will be found that a selection may be made from this group in which the value of this characteristic is in the range between .0001 for fused silica to about .0008 for beryllia for frequencies of about  $10^9$  c.p.s. The thermal coefficients of expansion of these materials range between about  $5 \times 10^{-7}$  for fused silica to about  $110 \times 10^{-7}$  for forsterite. The modulus of elasticity of the selected materials range between a low of  $10 \times 10^6$  for fused silica to a high of about  $40 \times 10^6$  for alumina. Of these six materials, the three that are preferred for microwave applications are fused silica, alumina and beryllia.

In conclusion it may be stated that any radio-frequency window of any configuration will be heated to some extent by various causes. It is important to conduct away as much of such heat as possible, regardless of the cause. It has been found that windows fabricated from beryllia, coated with titanium, and incorporated in metallic structures fabricated from oxygen-free, high conductivity copper which are also coated with titanium provide an almost ideal window package.

We claim:

1. In a radio-frequency device including an evacuated

section having juxtaposed metallic and dielectric portions with adjacent metallic and dielectric surfaces, said surfaces being exposed to vacuum within the evacuated section, means on said adjacent metallic and dielectric surfaces within the evacuated section providing a maximum coefficient of secondary electron emission ranging downwardly from about unity, said dielectric surface with said means thereon providing dielectric properties in said device.

10 2. The combination according to claim 1, in which said radio-frequency device comprises a metallic waveguide and a dielectric radio-frequency output window assembly, at least one surface of said window and the adjacent associated surface of the waveguide being exposed to vacuum within said evacuated section.

15 3. A radio-frequency device comprising an evacuated envelope having juxtaposed metallic and dielectric portions with metallic and dielectric surfaces exposed to vacuum, incident electrons, and electromagnetic energy within said envelope, said dielectric surface having means thereon providing a maximum coefficient of secondary electron emission ranging downwardly from about unity, said dielectric surface with said means thereon providing dielectric properties in said device.

20 25 4. A radio-frequency device according to claim 3 wherein said dielectric portion is an output window through which said electromagnetic energy passes.

#### References Cited

#### UNITED STATES PATENTS

|           |         |               |       |           |
|-----------|---------|---------------|-------|-----------|
| 3,059,142 | 10/1962 | Vaughan       | ----- | 333—98    |
| 2,821,659 | 1/1958  | Feinstein     | ----- | 315—39.77 |
| 2,955,229 | 10/1960 | Bondley       | ----- | 313—107 X |
| 2,958,804 | 11/1960 | Badger et al. | ----- | 315—5.39  |

HERMAN KARL SAALBACH, Primary Examiner.

SAXFIELD CHATMOH, Jr., Assistant Examiner.

#### U.S. Cl. X.R.

313—106; 315—5, 39, 39.53; 333—83